

# UNITED STATES PATENT OFFICE

CHRISTIAN EMIL BICHEL, OF HAMBURG, GERMANY.

## EXPLOSIVE.

No. 839,450.

Specification of Letters Patent.

Patented Dec. 25, 1906.

Application filed July 6, 1903. Serial No. 164,453.

To all whom it may concern:

Be it known that I, CHRISTIAN EMIL BICHEL, a subject of the German Emperor, residing at Hamburg, in the German Empire, have invented certain new and useful Improvements in Explosives, of which the following is a specification.

In manufacturing fire-damp-proof explosives and for enhancing the safety of the

same there have been successfully employed salts of ammonium, such as ammonium oxalate, ammonium acetate, ammonium sulfate, ammonium chlorid, and other similar salts. These admixtures, however, do not answer the desired purpose equally, and some of them exert an injurious effect upon the choke-damp, whereby part of the advantages that may be secured in other respects are lost. Therefore it has been necessary to add a nitrate of a metal of the alkalis, such as nitrate of potassium or nitrate of sodium, to the aforesaid salts for the purpose of improving the choke-damps and to successfully effect the reduction of the heat evolved at explosion. Very good results have been obtained, for example, by ammonium chlorid and nitrate of sodium, which form sodium chlorid on decomposition and which, on the one hand, reduce the amount of heat evolved by the detonation of the explosive to such a degree that they may ignite fire-damp as well as coal-dust only with great difficulty, while, on the other hand, they form no noxious or other gases which unpleasantly affect the breathing.

I have observed that owing to the high temperatures of dissociation ammonium chlorid and nitrate of sodium are converted into chlorid of sodium, said chlorid of sodium being vaporized and separated. Following this observation attempts have been made to obtain the same result by directly adding chlorids to the components of the explosives, and thereby reduce the temperature as well as to produce inert products of combustion. These experiments have been successful, and they prove that sodium chlorid may just as well be directly employed as salts that form sodium chlorid by double decomposition. To decide upon which of these methods to use depends upon the mechanical structure of the explosive, its specific gravity, its adaptability to the blast-holes and cartridges, and other circumstances. Thus in certain cases it may be advantageous to directly add chlorid of sodium to the explosive, while in other

cases chlorid of ammonium and nitrate of sodium or nitrate of potassium is preferably used.

It has been stated by official commissions in countries where fiery mines are worked that all explosives when fired in mixtures of pit-gas or coal-dust are liable to ignite this mixture if the quantity used for the shot is large enough.

It is the object of this invention to render most of the explosives safer against fire-damp and dry coal-dust than they are without the means mentioned herein. For example, the quantity of usual No. 1 dynamite (of seventy-five per cent. nitroglycerin and twenty-five per cent. of kieselguhr) of five grams regularly ignites a mixture of eight per cent. of fire-damp, (or a suitable quantity of benzin vapor, which gives the same effect,) whereas an explosive manufactured in accordance with this invention requires a quantity of more than five hundred grams without losing a great percentage of its strength, so that the safety is as five is to five hundred. The object of the invention therefore is to render the work in fiery mines safer.

The examples given hereinafter, recording, as they do, the results of actual experience, will confirm the above statements and the success of the invention:

1. Donarite of the following compositions: nitrate of ammonia, eighty per cent.; trinitrotoluol, twelve per cent.; flour, four per cent.; nitroglycerin, 3.8 per cent.; collodion, cotton, 0.2 per cent.

*Safety.*—Donarite alone, eighty-seven grams; ninety-five per cent. of donarite + five per cent. ammonium chlorid, one hundred and twenty-five grams; ninety per cent. of donarite + ten per cent. of ammonium chlorid, two hundred and fifty grams; eighty-six per cent. of donarite + 5.5 per cent. of ammonium chlorid and 8.5 per cent. sodium nitrate, four hundred and twenty-five grams. There was a reduction in the power displayed amounting to about eight per cent., while safety was enhanced five-fold.

2. Roburite of the following composition: nitrate of ammonia, 72.5 per cent.; binitrobenzol, twelve per cent.; potassium nitrate, ten per cent.; sulfate of ammonium, five per cent.; permanganate of potassium, 0.5 per cent.

*Safety.*—Roburite alone, three hundred and twenty-five grams; roburite with ammonium chlorid substituted for ammonium

sulfate, four hundred grams. At the same time there occurred an increase in the power.

3. An explosive hereinafter termed "X," of the following composition: nitroglycerin, 5 four per cent.; nitrate of ammonia, 75.5 per cent.; potassium nitrate, 9.5 per cent.; coal-dust, 0.5 per cent.; flour, 10.5 per cent.

*Safety.*—Explosive X alone, two hundred and fifty grams; ninety-five per cent. of explosive X + five per cent. of ammonium chlorid, four hundred grams; ninety-two per cent. of explosive X + eight per cent. of ammonium chlorid, five hundred grams.

The power displayed became reduced by 15 three per cent. when five per cent. of ammonium chlorid was added to the explosive.

The following table is intended to account for the influence exerted by ammonium chlorid when added to explosive X, the explosive of the aforesaid composition, viz:

| 25                                                              | Heat evolved at explosion in thermal units. | Duration of flame (or flash) in 1/1000 of a second. | Length of flame in centimeters. | Safety in grams. |
|-----------------------------------------------------------------|---------------------------------------------|-----------------------------------------------------|---------------------------------|------------------|
| Explosive X alone.....                                          | 863                                         | 0.403                                               | 54                              | 250              |
| 95 per cent. explosive X + 5 per cent. ammonium chlorid.....    | 781                                         | 0.262                                               | 45                              | 400              |
| 30 92 per cent. explosive X + 8 per cent. ammonium chlorid..... | 745                                         | 0.210                                               | 40                              | 500 and upward.  |

35 This table is based upon the method of investigation of explosives published in Part III, Vol. 50, of the journal *Zeitschrift für Berg-, Hütten- und Salinenwesen*. Hence it will be seen that by the addition of ammonium chlorid to the explosive X already containing 9.5 per cent. of potassium nitrate the number of thermal units, the time of flash, and the length of flame are reduced, while the safety from fire-damp is made to become 45 double what it was before—that is to say, without the separate addition of ammonium chlorid.

From the following examples it will be made clear that also very favorable results 50 will be obtained when chlorid of potassium

and chlorid of sodium are directly added to the explosives. So, for instance, an explosive composed of 25.30 per cent. of nitroglycerin, 0.70 per cent. of collodion-cotton, 6.90 per cent. of gelatinized glycerin, (obtained by dissolving one part of glue in 3.5 parts of glycerin,) 25.60 per cent. of sodium chlorid, and 41.50 per cent. of nitrate of ammonia has produced in Trauzl's lead block, an apparatus for testing strength of explosives, 6 (*vide* M. Eissler, *A Handbook on Modern Explosives*, London, 1897, page 176,) a distention of four hundred cubic centimeters and has proved a safety of five hundred and fifty grams, while an explosive consisting of twenty-two per cent. of nitroglycerin, 0.6 per cent. of collodion-cotton, eleven per cent. of potassium chlorid, 0.6 per cent. of sawdust, eight per cent. of gelatinized glycerin, (produced by dissolving one part of glue in three parts of glycerin,) and 57.8 per cent. of nitrate of ammonia has produced in Trauzl's lead block a distention of three hundred and forty-five cubic centimeters and has proved a safety of five hundred grams.

Having thus described my invention, what I claim as new therein, and desire to secure by Letters Patent, is—

1. A short-flame and quick-burning explosive containing a chlorid of an alkaline metal, 8 the vapor of which will damp the flame produced on explosion and enhance the safety of the explosive against the ignition of fire-damp and coal-dust-laden atmosphere, substantially as described.

2. A short-flame and quick-burning explosive containing sufficient chlorid of a metal of the alkalis to damp by the vapor of said chlorid the flame of the explosive, and enhance the safety of the explosive against the 9 ignition of fire-damp and coal-dust-laden atmosphere, substantially as described.

3. A short-flame and quick-burning explosive containing sufficient chlorid of sodium to damp the flame of the explosive, substantially as and for the purposes set forth.

CHRISTIAN EMIL BICHEL.

Witnesses:

ALEXANDER SPECHT,  
E. H. L. MUMMENHOFF.